

1

2,801,165

COBALT-BASE ALLOYS

James F. Baldwin, New York, N. Y., and Rey O. Sheets, Fairlawn, N. J., assignors to Coast Metals, Inc., Little Ferry, N. J., a corporation of Delaware

No Drawing. Application September 30, 1955,  
Serial No. 537,876

2 Claims. (Cl. 75—134)

This invention relates generally to high temperature alloys, but has reference more particularly to cobalt-base alloys of the Stellite type.

It has been generally known that increasing the tungsten content of cobalt-base alloys, such as alloys of the Stellite type, resulted in increased high temperature properties, but it was also thought that the improvement in high temperature properties would necessarily be uniform in character.

As the result of tests which have been conducted in connection with certain jet guided missile parts, we have discovered that the improvement in high temperature properties, resulting from the incorporation of increasingly larger amounts of tungsten in such cobalt-base alloys is not uniform, but that a marked and sudden increase in the improvement occurs when the tungsten reaches a value of about 18.75%, and that this improvement is effective up to a value of about 23.25% tungsten, beyond which there is no further improvement of consequence.

The aforesaid tests were conducted on lap joint test specimens made of stainless steel, with the cobalt base alloy of the present invention applied as a fillet on both sides of the lap joint. Precautions were taken to prevent any of the fillet material from flowing into the joint, and the fillets were maintained uniform as to dimensions in all of the test specimens.

The test specimens were heated to a temperature of 1600° F., and maintained at such temperature for 20 minutes, after which each specimen was subjected to a test to determine its ultimate strength at this temperature. In this way, assurance was had not only that each test piece had arrived at the desired temperature, but also that stresses which might have been produced by the welding operations incidental to formation of the fillets had been substantially eliminated. The results of these tests may be tabulated as follows:

| Alloy No. | Carbon | Chromium | Cobalt | Tungsten | Silicon | Iron | Ultimate Strength at 1,600° F., p. s. i. |
|-----------|--------|----------|--------|----------|---------|------|------------------------------------------|
| 1-----    | 1.98   | 28.24    | 49.60  | 17.12    | .20     | 1.70 | 29,500                                   |
| 2-----    | 2.21   | 28.70    | 48.00  | 18.08    | .38     | 1.70 | 32,000                                   |
| 3-----    | 1.89   | 26.44    | 50.32  | 19.72    | .38     | 1.40 | 49,400                                   |
| 4-----    | 1.80   | 30.45    | 44.68  | 18.86    | .37     | 1.40 | 47,700                                   |
| 5-----    | 1.80   | 26.39    | 48.50  | 19.94    | .40     | 1.20 | 46,000                                   |
| 6-----    | 1.82   | 28.00    | 44.00  | 22.55    | .42     | 1.50 | 50,600                                   |

In the aforesaid alloys, the balance of the alloy, in each case, consists of small and inconsequential amounts of residual or trace elements, such as manganese, sulphur, and vanadium. Vanadium is usually added to obtain grain refinement in the alloy, and when thus used, may be present in amounts up to about 2%. It improves the

2

general physical properties of the alloy to some extent, but does not affect its high temperature properties.

It was found that increasing the tungsten content beyond 23.25% did not improve the high temperature properties to any appreciable extent, yet worsened materially the problems of welding and casting.

Based on the aforesaid tests and other factors, the following analysis range covers all alloys coming within the scope of the invention:

|    |          |               |
|----|----------|---------------|
| 10 | Carbon   | 1.35-2.25%.   |
|    | Chromium | 26-30%.       |
|    | Cobalt   | 44-51%.       |
|    | Tungsten | 18.75-23.25%. |
|    | Silicon  | 1.75% max.    |
|    | Iron     | 3% max.       |

The aforesaid alloy may also contain small and inconsequential amounts of residual or trace elements, such as manganese, sulphur and vanadium, and such residual amounts are contemplated as falling within the scope of the expression "the balance being substantially all iron," as used in the appended claims.

The hardness values, at room temperatures, of alloys within the aforesaid analysis range, were between 45 Rockwell C and 62 Rockwell C. It was found that increasing the carbon content of the alloy produced hardnesses above 62 Rockwell C, but increased brittleness of the alloy, and that alloys with hardnesses below 45 Rockwell C were not sufficiently resistant to wear or abrasion.

20 The alloys of the present invention are especially resistant to fatigue at high temperatures, and have been found to be especially useful for applications for which cobalt-chromium-tungsten alloys of conventional analysis ranges have been found to be inadequate.

30 The alloys may be used either in the form of castings, or as weld rods for the hard surfacing of parts which require the properties which are inherent in these alloys.

It may be noted that in contradistinction to known alloys of this type, molybdenum is not substitutable for 40 any part of the tungsten of the alloys of this invention, without materially altering the properties of the alloy, and that nickel is not substitutable for any part of the cobalt.

35 It will be understood that slight changes may be made in the alloy without departing from the scope of the invention, as defined by the appended claims.

Having thus described our invention, we claim:

1. An alloy which is especially resistant to fatigue at 45 high temperatures, said alloy consisting of carbon in amounts of from about 1.35% to about 2.25%, chromium in amounts of from about 26% to about 30%, cobalt in amounts of from about 44% to about 51%, tungsten in amounts of from about 18.75% to about 23.25%, and silicon up to a maximum of about 1.75%, the balance of the alloy being substantially all iron, but not to exceed about 3%.

2. An alloy, as defined in claim 1, having a Rockwell C hardness of from about 45 to about 62.

60 References Cited in the file of this patent

UNITED STATES PATENTS

|           |            |               |
|-----------|------------|---------------|
| 2,048,706 | Pfanstiehl | July 28, 1936 |
| 2,235,232 | McElroy    | Mar. 18, 1941 |
| 2,299,871 | Baird      | Oct. 27, 1942 |
| 2,309,372 | Wissler    | Jan. 26, 1943 |
| 2,551,170 | Schmucker  | May 1, 1951   |
| 2,553,609 | Schmidt    | May 22, 1951  |